



US010190263B2

(12) **United States Patent**  
Ramaratnam et al.

(10) **Patent No.:** US 10,190,263 B2  
(45) **Date of Patent:** Jan. 29, 2019

(54) **SOFT THROUGH AIR DRIED TISSUE**

(71) Applicant: **FIRST QUALITY TISSUE, LLC**,  
Great Neck, NY (US)

(72) Inventors: **Karthik Ramaratnam**, Anderson, SC  
(US); **Byrd Tyler Miller, IV**, Easley,  
SC (US); **Shane Ervin Hayes**,  
Anderson, SC (US); **James E. Sealey,  
II**, Belton, SC (US)

(73) Assignee: **First Quality Tissue, LLC**, Great  
Neck, NY (US)

(\*) Notice: Subject to any disclaimer, the term of this  
patent is extended or adjusted under 35  
U.S.C. 154(b) by 0 days.

(21) Appl. No.: **15/614,156**

(22) Filed: **Jun. 5, 2017**

(65) **Prior Publication Data**

US 2017/0268178 A1 Sep. 21, 2017

**Related U.S. Application Data**

(60) Division of application No. 15/182,391, filed on Jun.  
14, 2016, now Pat. No. 9,702,090, which is a  
(Continued)

(51) **Int. Cl.**  
**D21H 27/38** (2006.01)  
**D21H 27/00** (2006.01)

(Continued)

(52) **U.S. Cl.**  
CPC ..... **D21H 27/38** (2013.01); **D21F 11/145**  
(2013.01); **D21H 11/04** (2013.01); **D21H  
21/14** (2013.01);

(Continued)

(58) **Field of Classification Search**

CPC ..... D21J 1/16; D21H 27/30; D21H 27/38;  
D21H 27/002; D21H 21/18; D21H 21/20;  
D21F 1/66

(Continued)

(56) **References Cited**

U.S. PATENT DOCUMENTS

2,919,467 A 1/1960 Mercer  
2,926,154 A 2/1960 Keim

(Continued)

FOREIGN PATENT DOCUMENTS

CA 2168894 A1 8/1997  
CA 2795139 A1 10/2011

(Continued)

OTHER PUBLICATIONS

Written Opinion of International Searching Authority for PCT/US15/  
62483 dated May 6, 2016.

(Continued)

*Primary Examiner* — Mark Halpern

(74) *Attorney, Agent, or Firm* — Amster, Rothstein &  
Ebenstein LLP

(57) **ABSTRACT**

A process for manufacturing tissue including providing a first pulp mix, delivering a wet-end additive to the first pulp mix at a first point in the process, forming a tissue web comprising the first pulp mix after the first point in the process, monitoring the tissue web for breaks and preventing delivery of the wet-end additive to the first pulp mix at the first point in response to detecting a break in the monitoring step. In an exemplary embodiment, a switching valve is used to control delivery of the wet-end additive to the first pulp mix.

**6 Claims, 3 Drawing Sheets**



**Related U.S. Application Data**

continuation of application No. 14/534,631, filed on Nov. 6, 2014, now Pat. No. 9,382,666, which is a division of application No. 13/837,685, filed on Mar. 15, 2013, now Pat. No. 8,968,517.

(60) Provisional application No. 61/679,337, filed on Aug. 3, 2012.

**(51) Int. Cl.**

**D21H 27/40** (2006.01)  
**D21F 11/14** (2006.01)  
**D21H 11/04** (2006.01)  
**D21H 21/18** (2006.01)  
**D21H 21/20** (2006.01)  
**D21H 21/14** (2006.01)  
**D21H 27/30** (2006.01)

**(52) U.S. Cl.**

CPC ..... **D21H 21/18** (2013.01); **D21H 21/20** (2013.01); **D21H 27/002** (2013.01); **D21H 27/004** (2013.01); **D21H 27/005** (2013.01); **D21H 27/008** (2013.01); **D21H 27/30** (2013.01); **D21H 27/40** (2013.01)

**(58) Field of Classification Search**

USPC ..... 162/127, 198, 259  
 See application file for complete search history.

**(56) References Cited****U.S. PATENT DOCUMENTS**

|             |         |                  |             |         |                          |
|-------------|---------|------------------|-------------|---------|--------------------------|
| 3,026,231 A | 3/1962  | Chavannes        | 3,877,510 A | 4/1975  | Tegtmeier et al.         |
| 3,049,469 A | 8/1962  | Davison          | 3,905,863 A | 9/1975  | Ayers                    |
| 3,058,873 A | 10/1962 | Keim et al.      | 3,911,173 A | 10/1975 | Sprague, Jr.             |
| 3,066,066 A | 11/1962 | Keim et al.      | 3,974,025 A | 8/1976  | Ayers                    |
| 3,097,994 A | 7/1963  | Dickens et al.   | 3,994,771 A | 11/1976 | Morgan, Jr. et al.       |
| 3,125,552 A | 3/1964  | Loshack et al.   | 3,998,690 A | 12/1976 | Lyness et al.            |
| 3,143,150 A | 8/1964  | Buchanan         | 4,038,008 A | 7/1977  | Larsen                   |
| 3,186,900 A | 6/1965  | De Young         | 4,075,382 A | 2/1978  | Chapman et al.           |
| 3,197,427 A | 7/1965  | Schmalz          | 4,088,528 A | 5/1978  | Berger et al.            |
| 3,224,986 A | 12/1965 | Butler et al.    | 4,098,632 A | 7/1978  | Sprague, Jr.             |
| 3,224,990 A | 12/1965 | Babcock          | 4,102,737 A | 7/1978  | Morton                   |
| 3,227,615 A | 1/1966  | Korden           | 4,129,528 A | 12/1978 | Petrovich et al.         |
| 3,227,671 A | 1/1966  | Keim             | 4,147,586 A | 4/1979  | Petrovich et al.         |
| 3,239,491 A | 3/1966  | Tsou et al.      | 4,184,519 A | 1/1980  | McDonald et al.          |
| 3,240,664 A | 3/1966  | Earle, Jr.       | 4,190,692 A | 2/1980  | Larsen                   |
| 3,240,761 A | 3/1966  | Keim et al.      | 4,191,609 A | 3/1980  | Trokan                   |
| 3,248,280 A | 4/1966  | Hyland, Jr.      | 4,252,761 A | 2/1981  | Schoggen et al.          |
| 3,250,664 A | 5/1966  | Conte et al.     | 4,320,162 A | 3/1982  | Schulz                   |
| 3,252,181 A | 5/1966  | Hureau           | 4,331,510 A | 5/1982  | Wells                    |
| 3,301,746 A | 1/1967  | Sanford et al.   | 4,382,987 A | 5/1983  | Smart                    |
| 3,311,594 A | 3/1967  | Earle, Jr.       | 4,440,597 A | 4/1984  | Wells et al.             |
| 3,329,657 A | 7/1967  | Strazdins et al. | 4,501,862 A | 2/1985  | Keim                     |
| 3,332,834 A | 7/1967  | Reynolds, Jr.    | 4,507,351 A | 3/1985  | Johnson et al.           |
| 3,332,901 A | 7/1967  | Keim             | 4,514,345 A | 4/1985  | Johnson et al.           |
| 3,352,833 A | 11/1967 | Earle, Jr.       | 4,515,657 A | 5/1985  | Maslanka                 |
| 3,384,692 A | 5/1968  | Galt et al.      | 4,528,239 A | 7/1985  | Trokan                   |
| 3,414,459 A | 12/1968 | Wells            | 4,529,480 A | 7/1985  | Trokan                   |
| 3,442,754 A | 5/1969  | Espy             | 4,537,657 A | 8/1985  | Keim                     |
| 3,459,697 A | 8/1969  | Goldberg et al.  | 4,545,857 A | 10/1985 | Wells                    |
| 3,473,576 A | 10/1969 | Amneus           | 4,637,859 A | 1/1987  | Trokan                   |
| 3,483,077 A | 12/1969 | Aldrich          | 4,678,590 A | 7/1987  | Nakamura et al.          |
| 3,545,165 A | 12/1970 | Greenwell        | 4,714,736 A | 12/1987 | Juhl et al.              |
| 3,556,932 A | 1/1971  | Coscia et al.    | 4,770,920 A | 9/1988  | Larsonneur               |
| 3,573,164 A | 3/1971  | Friedberg et al. | 4,780,357 A | 10/1988 | Akao                     |
| 3,609,126 A | 9/1971  | Asao et al.      | 4,808,467 A | 2/1989  | Suskind et al.           |
| 3,666,609 A | 5/1972  | Kalwaites et al. | 4,836,894 A | 6/1989  | Chance et al.            |
| 3,672,949 A | 6/1972  | Brown            | 4,849,054 A | 7/1989  | Klowak                   |
| 3,672,950 A | 6/1972  | Murphy et al.    | 4,885,202 A | 12/1989 | Lloyd et al.             |
| 3,773,290 A | 11/1973 | Mowery           | 4,891,249 A | 1/1990  | McIntyre                 |
| 3,778,339 A | 12/1973 | Williams et al.  | 4,909,284 A | 3/1990  | Kositake                 |
| 3,813,362 A | 5/1974  | Coscia et al.    | 4,949,668 A | 8/1990  | Heindel et al.           |
| 3,855,158 A | 12/1974 | Petrovich et al. | 4,949,688 A | 8/1990  | Bayless                  |
|             |         |                  | 4,983,256 A | 1/1991  | Comette et al.           |
|             |         |                  | 4,996,091 A | 2/1991  | McIntyre                 |
|             |         |                  | 5,059,282 A | 10/1991 | Ampulski et al.          |
|             |         |                  | 5,143,776 A | 9/1992  | Givens                   |
|             |         |                  | 5,149,401 A | 9/1992  | Langevin et al.          |
|             |         |                  | 5,152,874 A | 10/1992 | Keller                   |
|             |         |                  | 5,211,813 A | 5/1993  | Sawley et al.            |
|             |         |                  | 5,239,047 A | 8/1993  | Devore et al.            |
|             |         |                  | 5,279,098 A | 1/1994  | Fukuda                   |
|             |         |                  | 5,281,306 A | 1/1994  | Kakiuchi et al.          |
|             |         |                  | 5,334,289 A | 8/1994  | Trokan et al.            |
|             |         |                  | 5,347,795 A | 9/1994  | Fukuda                   |
|             |         |                  | 5,397,435 A | 3/1995  | Ostendorf et al.         |
|             |         |                  | 5,399,412 A | 3/1995  | Sudall et al.            |
|             |         |                  | 5,405,501 A | 4/1995  | Phan et al.              |
|             |         |                  | 5,409,572 A | 4/1995  | Kershaw et al.           |
|             |         |                  | 5,429,686 A | 7/1995  | Chiu et al.              |
|             |         |                  | 5,439,559 A | 8/1995  | Crouse                   |
|             |         |                  | 5,447,012 A | 9/1995  | Kovacs et al.            |
|             |         |                  | 5,470,436 A | 11/1995 | Wagle et al.             |
|             |         |                  | 5,487,313 A | 1/1996  | Johnson                  |
|             |         |                  | 5,509,913 A | 4/1996  | Yeo                      |
|             |         |                  | 5,510,002 A | 4/1996  | Hermans et al.           |
|             |         |                  | 5,529,665 A | 6/1996  | Kaun                     |
|             |         |                  | 5,581,906 A | 12/1996 | Ensign et al.            |
|             |         |                  | 5,591,147 A | 1/1997  | Couture-Dorschner et al. |
|             |         |                  | 5,607,551 A | 3/1997  | Farrington, Jr. et al.   |
|             |         |                  | 5,611,890 A | 3/1997  | Vinson et al.            |
|             |         |                  | 5,628,876 A | 5/1997  | Ayers et al.             |
|             |         |                  | 5,635,028 A | 6/1997  | Vinson et al.            |
|             |         |                  | 5,649,916 A | 7/1997  | DiPalma et al.           |
|             |         |                  | 5,671,897 A | 9/1997  | Ogg et al.               |
|             |         |                  | 5,672,248 A | 9/1997  | Wendt et al.             |
|             |         |                  | 5,679,222 A | 10/1997 | Rasch et al.             |
|             |         |                  | 5,685,428 A | 11/1997 | Herbers et al.           |
|             |         |                  | 5,728,268 A | 3/1998  | Weisman et al.           |
|             |         |                  | 5,746,887 A | 5/1998  | Wendt et al.             |

| (56)                  | References Cited |                        |              |         |                    |  |
|-----------------------|------------------|------------------------|--------------|---------|--------------------|--|
| U.S. PATENT DOCUMENTS |                  |                        |              |         |                    |  |
| 5,753,067 A           | 5/1998           | Fukuda et al.          | 7,311,853 B2 | 12/2007 | Vinson et al.      |  |
| 5,772,845 A           | 6/1998           | Farrington, Jr. et al. | 7,328,550 B2 | 2/2008  | Flodding et al.    |  |
| 5,806,569 A           | 9/1998           | Gulya et al.           | 7,339,378 B2 | 3/2008  | Han et al.         |  |
| 5,827,384 A           | 10/1998          | Canfield et al.        | 7,419,569 B2 | 9/2008  | Hermans            |  |
| 5,832,962 A           | 11/1998          | Kaufman et al.         | 7,427,434 B2 | 9/2008  | Busam              |  |
| 5,846,380 A           | 12/1998          | Van Phan et al.        | 7,431,801 B2 | 10/2008 | Conn et al.        |  |
| 5,855,738 A           | 1/1999           | Weisman et al.         | 7,432,309 B2 | 10/2008 | Vinson             |  |
| 5,858,554 A           | 1/1999           | Neal et al.            | 7,442,278 B2 | 10/2008 | Murray et al.      |  |
| 5,865,396 A           | 2/1999           | Ogg et al.             | 7,452,447 B2 | 11/2008 | Duan et al.        |  |
| 5,865,950 A           | 2/1999           | Vinson et al.          | 7,476,293 B2 | 1/2009  | Herman et al.      |  |
| 5,893,965 A           | 4/1999           | Trokhman et al.        | 7,494,563 B2 | 2/2009  | Edwards et al.     |  |
| 5,913,765 A           | 6/1999           | Burgess et al.         | 7,510,631 B2 | 3/2009  | Scherb et al.      |  |
| 5,942,085 A           | 8/1999           | Neal et al.            | 7,513,975 B2 | 4/2009  | Burma              |  |
| 5,944,954 A           | 8/1999           | Vinson et al.          | 7,563,344 B2 | 7/2009  | Beuther            |  |
| 5,948,210 A           | 9/1999           | Huston                 | 7,582,187 B2 | 9/2009  | Scherb et al.      |  |
| 5,980,691 A           | 11/1999          | Weisman et al.         | 7,611,607 B2 | 11/2009 | Mullally et al.    |  |
| 6,036,139 A           | 3/2000           | Ogg                    | 7,622,020 B2 | 11/2009 | Awofeso            |  |
| 6,039,838 A           | 3/2000           | Kaufman et al.         | 7,662,462 B2 | 2/2010  | Noda               |  |
| 6,048,938 A           | 4/2000           | Neal et al.            | 7,670,678 B2 | 3/2010  | Phan               |  |
| 6,060,149 A           | 5/2000           | Nissing et al.         | 7,683,126 B2 | 3/2010  | Neal et al.        |  |
| 6,106,670 A           | 8/2000           | Weisman et al.         | 7,686,923 B2 | 3/2010  | Scherb et al.      |  |
| 6,149,769 A           | 11/2000          | Mohammadi et al.       | 7,687,140 B2 | 3/2010  | Manifold et al.    |  |
| 6,162,327 A           | 12/2000          | Batra et al.           | 7,691,230 B2 | 4/2010  | Scherb et al.      |  |
| 6,162,329 A           | 12/2000          | Vinson et al.          | 7,744,722 B1 | 6/2010  | Tucker et al.      |  |
| 6,187,138 B1          | 2/2001           | Neal et al.            | 7,744,726 B2 | 6/2010  | Scherb et al.      |  |
| 6,200,419 B1          | 3/2001           | Phan                   | 7,799,382 B2 | 9/2010  | Payne et al.       |  |
| 6,203,667 B1          | 3/2001           | Huhtelin               | 7,811,418 B2 | 10/2010 | Klerelid et al.    |  |
| 6,207,734 B1          | 3/2001           | Vinson et al.          | 7,815,978 B2 | 10/2010 | Davenport et al.   |  |
| 6,231,723 B1          | 5/2001           | Kanitz et al.          | 7,823,366 B2 | 11/2010 | Schoeneck          |  |
| 6,287,426 B1          | 9/2001           | Edwards et al.         | 7,842,163 B2 | 11/2010 | Nickel et al.      |  |
| 6,303,233 B1          | 10/2001          | Amon et al.            | 7,867,361 B2 | 1/2011  | Salaam et al.      |  |
| 6,319,362 B1          | 11/2001          | Huhtelin et al.        | 7,871,692 B2 | 1/2011  | Morin et al.       |  |
| 6,344,111 B1          | 2/2002           | Wilhelm                | 7,887,673 B2 | 2/2011  | Andersson et al.   |  |
| 6,420,013 B1          | 7/2002           | Vinson et al.          | 7,905,989 B2 | 3/2011  | Scherb et al.      |  |
| 6,420,100 B1          | 7/2002           | Trokhman et al.        | 7,914,866 B2 | 3/2011  | Shannon et al.     |  |
| 6,423,184 B2          | 7/2002           | Vahatalo et al.        | 7,931,781 B2 | 4/2011  | Scherb et al.      |  |
| 6,458,246 B1          | 10/2002          | Kanitz et al.          | 7,951,269 B2 | 5/2011  | Herman et al.      |  |
| 6,464,831 B1          | 10/2002          | Trokhman et al.        | 7,955,549 B2 | 6/2011  | Noda               |  |
| 6,473,670 B1          | 10/2002          | Huhtelin               | 7,959,764 B2 | 6/2011  | Ringer et al.      |  |
| 6,521,089 B1          | 2/2003           | Griech et al.          | 7,972,475 B2 | 7/2011  | Chen et al.        |  |
| 6,537,407 B1          | 3/2003           | Law et al.             | 7,989,058 B2 | 8/2011  | Manifold et al.    |  |
| 6,547,928 B2          | 4/2003           | Barnholtz et al.       | 8,034,463 B2 | 10/2011 | Leimbach et al.    |  |
| 6,551,453 B2          | 4/2003           | Weisman et al.         | 8,051,629 B2 | 11/2011 | Pazdemik et al.    |  |
| 6,551,691 B1          | 4/2003           | Hoeft et al.           | 8,075,739 B2 | 12/2011 | Scherb et al.      |  |
| 6,572,722 B1          | 6/2003           | Pratt                  | 8,092,652 B2 | 1/2012  | Scherb et al.      |  |
| 6,579,416 B1          | 6/2003           | Vinson et al.          | 8,118,979 B2 | 2/2012  | Herman et al.      |  |
| 6,602,454 B2          | 8/2003           | McGuire et al.         | 8,147,649 B1 | 4/2012  | Tucker et al.      |  |
| 6,607,637 B1          | 8/2003           | Vinson et al.          | 8,152,959 B2 | 4/2012  | Elony et al.       |  |
| 6,610,173 B1          | 8/2003           | Lindsay et al.         | 8,196,314 B2 | 6/2012  | Munch              |  |
| 6,613,194 B2          | 9/2003           | Kanitz et al.          | 8,216,427 B2 | 7/2012  | Klerelid et al.    |  |
| 6,660,362 B1          | 12/2003          | Lindsay et al.         | 8,236,135 B2 | 8/2012  | Prodoehl et al.    |  |
| 6,673,202 B2          | 1/2004           | Burazin                | 8,303,773 B2 | 11/2012 | Scherb et al.      |  |
| 6,701,637 B2          | 5/2004           | Lindsay et al.         | 8,382,956 B2 | 2/2013  | Boechat et al.     |  |
| 6,755,939 B2          | 6/2004           | Vinson et al.          | 8,402,673 B2 | 3/2013  | Da Silva et al.    |  |
| 6,773,647 B2          | 8/2004           | McGuire et al.         | 8,409,404 B2 | 4/2013  | Harper et al.      |  |
| 6,797,117 B1          | 9/2004           | McKay et al.           | 8,435,384 B2 | 5/2013  | Da Silva et al.    |  |
| 6,808,599 B2          | 10/2004          | Burazin                | 8,440,055 B2 | 5/2013  | Scherb et al.      |  |
| 6,821,386 B2          | 11/2004          | Weisman et al.         | 8,445,032 B2 | 5/2013  | Topolkaraev et al. |  |
| 6,821,391 B2          | 11/2004          | Scherb et al.          | 8,454,800 B2 | 6/2013  | Mourad et al.      |  |
| 6,827,818 B2          | 12/2004          | Farrington, Jr. et al. | 8,470,133 B2 | 6/2013  | Cunnane et al.     |  |
| 6,863,777 B2          | 3/2005           | Kanitz et al.          | 8,506,756 B2 | 8/2013  | Denis et al.       |  |
| 6,896,767 B2          | 5/2005           | Wilhelm                | 8,544,184 B2 | 10/2013 | Da Silva et al.    |  |
| 6,939,443 B2          | 9/2005           | Ryan et al.            | 8,574,211 B2 | 11/2013 | Morita             |  |
| 6,998,017 B2          | 2/2006           | Lindsay et al.         | 8,580,083 B2 | 11/2013 | Boechat et al.     |  |
| 6,998,024 B2          | 2/2006           | Burazin                | 8,728,277 B2 | 5/2014  | Boechat et al.     |  |
| 7,005,043 B2          | 2/2006           | Toney et al.           | 8,758,569 B2 | 6/2014  | Aberg et al.       |  |
| 7,014,735 B2          | 3/2006           | Kramer et al.          | 8,771,466 B2 | 7/2014  | Denis et al.       |  |
| 7,105,465 B2          | 9/2006           | Patel et al.           | 8,801,903 B2 | 8/2014  | Mourad et al.      |  |
| 7,155,876 B2          | 1/2007           | VanderTuin et al.      | 8,815,057 B2 | 8/2014  | Eberhardt et al.   |  |
| 7,157,389 B2          | 1/2007           | Branham et al.         | 8,822,009 B2 | 9/2014  | Riviere et al.     |  |
| 7,182,837 B2          | 2/2007           | Chen et al.            | 8,968,517 B2 | 3/2015  | Ramaratnam et al.  |  |
| 7,194,788 B2          | 3/2007           | Clark et al.           | 8,980,062 B2 | 3/2015  | Karlsson et al.    |  |
| 7,235,156 B2          | 6/2007           | Baggot                 | 9,005,710 B2 | 4/2015  | Jones et al.       |  |
| 7,269,929 B2          | 9/2007           | VanderTuin et al.      | D734,617 S   | 7/2015  | Seitzinger et al.  |  |
| 7,294,230 B2          | 11/2007          | Flugge-Berendes et al. | 9,095,477 B2 | 8/2015  | Yamaguchi          |  |
|                       |                  |                        | D738,633 S   | 9/2015  | Seitzinger et al.  |  |

| (56)                  | References Cited |                        |                 |           |                    |  |
|-----------------------|------------------|------------------------|-----------------|-----------|--------------------|--|
| U.S. PATENT DOCUMENTS |                  |                        |                 |           |                    |  |
| 9,382,666 B2          | 7/2016           | Ramaratnam et al.      | 2009/0020248 A1 | 1/2009    | Sumnicht et al.    |  |
| 9,506,203 B2          | 11/2016          | Ramaratnam et al.      | 2009/0056892 A1 | 3/2009    | Rekoske            |  |
| 9,580,872 B2          | 2/2017           | Ramaratnam et al.      | 2009/0061709 A1 | 3/2009    | Nakai et al.       |  |
| 9,702,089 B2          | 7/2017           | Ramaratnam et al.      | 2009/0205797 A1 | 8/2009    | Fernandes et al.   |  |
| 9,702,090 B2          | 7/2017           | Ramaratnam et al.      | 2009/0218056 A1 | 9/2009    | Manifold et al.    |  |
| 9,719,213 B2          | 8/2017           | Miller, IV et al.      | 2010/0065234 A1 | 3/2010    | Klerelid et al.    |  |
| 9,725,853 B2          | 8/2017           | Ramaratnam et al.      | 2010/0119779 A1 | 5/2010    | Ostendorf et al.   |  |
| 2001/0018068 A1       | 8/2001           | Lorenzi et al.         | 2010/0224338 A1 | 9/2010    | Harper et al.      |  |
| 2002/0028230 A1       | 3/2002           | Eichhorn et al.        | 2010/0230064 A1 | 9/2010    | Eagles et al.      |  |
| 2002/0060049 A1       | 5/2002           | Kanitz et al.          | 2010/0236034 A1 | 9/2010    | Eagles et al.      |  |
| 2002/0061386 A1       | 5/2002           | Carson et al.          | 2010/0239825 A1 | 9/2010    | Sheehan et al.     |  |
| 2002/0098317 A1       | 7/2002           | Jaschinski et al.      | 2010/0272965 A1 | 10/2010   | Schinkoreit et al. |  |
| 2002/0110655 A1       | 8/2002           | Seth                   | 2011/0027545 A1 | 2/2011    | Harlacher et al.   |  |
| 2002/0115194 A1       | 8/2002           | Lange et al.           | 2011/0180223 A1 | 7/2011    | Klerelid et al.    |  |
| 2002/0125606 A1       | 9/2002           | McGuire et al.         | 2011/0189435 A1 | 8/2011    | Manifold et al.    |  |
| 2003/0024674 A1       | 2/2003           | Kanitz et al.          | 2011/0189442 A1 | 8/2011    | Manifold et al.    |  |
| 2003/0056911 A1       | 3/2003           | Hermans et al.         | 2011/0206913 A1 | 8/2011    | Manifold et al.    |  |
| 2003/0056917 A1       | 3/2003           | Jimenez                | 2011/0223381 A1 | 9/2011    | Sauter et al.      |  |
| 2003/0070781 A1       | 4/2003           | Hermans et al.         | 2011/0253329 A1 | 10/2011   | Manifold et al.    |  |
| 2003/0114071 A1       | 6/2003           | Everhart et al.        | 2011/0265967 A1 | 11/2011   | Van Phan           |  |
| 2003/0159401 A1       | 8/2003           | Sorensson et al.       | 2011/0303379 A1 | 12/2011   | Boechat et al.     |  |
| 2003/0188843 A1       | 10/2003          | Kanitz et al.          | 2012/0144611 A1 | 6/2012    | Baker et al.       |  |
| 2003/0218274 A1       | 11/2003          | Boutilier et al.       | 2012/0152475 A1 | 6/2012    | Edwards et al.     |  |
| 2004/0118531 A1       | 6/2004           | Shannon et al.         | 2012/0177888 A1 | 7/2012    | Escafere et al.    |  |
| 2004/0123963 A1       | 7/2004           | Chen et al.            | 2012/0244241 A1 | 9/2012    | McNeil             |  |
| 2004/0126601 A1       | 7/2004           | Kramer et al.          | 2012/0267063 A1 | 10/2012   | Klerelid et al.    |  |
| 2004/0126710 A1       | 7/2004           | Hill et al.            | 2012/0297560 A1 | 11/2012   | Zwick et al.       |  |
| 2004/0168784 A1       | 9/2004           | Duan et al.            | 2013/0008135 A1 | 1/2013    | Moore et al.       |  |
| 2004/0173333 A1       | 9/2004           | Hermans et al.         | 2013/0029105 A1 | 1/2013    | Miller et al.      |  |
| 2004/0234804 A1       | 11/2004          | Liu et al.             | 2013/0029106 A1 | 1/2013    | Lee et al.         |  |
| 2005/0016704 A1*      | 1/2005           | Huhtelin .....         | D21F 1/66       | 12/2013   | Espinosa et al.    |  |
|                       |                  |                        | 162/198         |           |                    |  |
| 2005/0069679 A1       | 3/2005           | Stelljes et al.        | 2013/0327487 A1 | 1/2014    | Sheehan            |  |
| 2005/0069680 A1       | 3/2005           | Stelljes et al.        | 2014/0004307 A1 | 1/2014    | Ramaratnam et al.  |  |
| 2005/0098281 A1       | 5/2005           | Schulz et al.          | 2014/0041820 A1 | 2/2014    | Boechat et al.     |  |
| 2005/0112115 A1       | 5/2005           | Khan                   | 2014/0041822 A1 | 2/2014    | Boechat et al.     |  |
| 2005/0123726 A1       | 6/2005           | Broering et al.        | 2014/0050890 A1 | 2/2014    | Zwick et al.       |  |
| 2005/0130536 A1       | 6/2005           | Siebers et al.         | 2014/0053994 A1 | 2/2014    | Manifold et al.    |  |
| 2005/0136222 A1       | 6/2005           | Hada et al.            | 2014/0096924 A1 | 4/2014    | Rekokske et al.    |  |
| 2005/0148257 A1       | 7/2005           | Hermans et al.         | 2014/0182798 A1 | 7/2014    | Polat et al.       |  |
| 2005/0150626 A1       | 7/2005           | Kanitz et al.          | 2014/0242320 A1 | 8/2014    | McNeil et al.      |  |
| 2005/0166551 A1       | 8/2005           | Keane et al.           | 2014/0272269 A1 | 9/2014    | Hansen             |  |
| 2005/0241786 A1       | 11/2005          | Edwards et al.         | 2014/0272747 A1 | 9/2014    | Ciurkot            |  |
| 2005/0241788 A1       | 11/2005          | Baggot et al.          | 2014/0284237 A1 | 9/2014    | Gosset             |  |
| 2005/0252626 A1       | 11/2005          | Chen et al.            | 2014/0360519 A1 | 12/2014   | George et al.      |  |
| 2005/0280184 A1       | 12/2005          | Sayers et al.          | 2015/0059995 A1 | 3/2015    | Ramaratnam et al.  |  |
| 2005/0287340 A1       | 12/2005          | Morelli et al.         | 2015/0102526 A1 | 4/2015    | Ward et al.        |  |
| 2006/0005916 A1       | 1/2006           | Stelljes et al.        | 2015/0129145 A1 | 5/2015    | Chou et al.        |  |
| 2006/0013998 A1       | 1/2006           | Stelljes et al.        | 2015/0211179 A1 | 7/2015    | Alias et al.       |  |
| 2006/0019567 A1       | 1/2006           | Sayers                 | 2015/0241788 A1 | 8/2015    | Yamaguchi          |  |
| 2006/0083899 A1       | 4/2006           | Burazin et al.         | 2015/0330029 A1 | 11/2015   | Ramaratnam et al.  |  |
| 2006/0093788 A1       | 5/2006           | Behm et al.            | 2016/0060811 A1 | 3/2016    | Riding et al.      |  |
| 2006/0113049 A1       | 6/2006           | Knobloch et al.        | 2016/0090692 A1 | 3/2016    | Eagles et al.      |  |
| 2006/0130986 A1       | 6/2006           | Flugge-Berendes et al. | 2016/0090693 A1 | 3/2016    | Eagles et al.      |  |
| 2006/0194022 A1       | 8/2006           | Boutilier et al.       | 2016/0130762 A1 | 5/2016    | Ramaratnam et al.  |  |
| 2006/0269706 A1       | 11/2006          | Shannon et al.         | 2016/0145810 A1 | 5/2016    | Miller, IV et al.  |  |
| 2007/0020315 A1       | 1/2007           | Shannon et al.         | 2016/0159007 A1 | 6/2016    | Miller, IV et al.  |  |
| 2007/0131366 A1       | 6/2007           | Underhill et al.       | 2016/0160448 A1 | 6/2016    | Miller, IV et al.  |  |
| 2007/0137813 A1       | 6/2007           | Nickel et al.          | 2016/0185041 A1 | 6/2016    | Topolkaraev et al. |  |
| 2007/0137814 A1       | 6/2007           | Gao                    | 2016/0185050 A1 | 6/2016    | Topolkaraev et al. |  |
| 2007/0170610 A1       | 7/2007           | Payne et al.           | 2016/0273168 A1 | 9/2016    | Ramaratnam et al.  |  |
| 2007/0240842 A1       | 10/2007          | Scherb et al.          | 2016/0273169 A1 | 9/2016    | Ramaratnam et al.  |  |
| 2007/0251659 A1       | 11/2007          | Fernandes et al.       | 2016/0289897 A1 | 10/2016   | Ramaratnam et al.  |  |
| 2007/0251660 A1       | 11/2007          | Walkenhaus et al.      | 2016/0289898 A1 | 10/2016   | Ramaratnam et al.  |  |
| 2007/0267157 A1       | 11/2007          | Kanitz et al.          | 2017/0044717 A1 | 2/2017    | Quigley            |  |
| 2007/0272381 A1       | 11/2007          | Elony et al.           | 2017/0101741 A1 | 4/2017    | Sealey et al.      |  |
| 2007/0275866 A1       | 11/2007          | Dykstra                | 2017/0167082 A1 | 6/2017    | Ramaratnam et al.  |  |
| 2007/0298221 A1       | 12/2007          | Vinson                 | 2017/0226698 A1 | 8/2017    | LeBrun et al.      |  |
| 2008/0035289 A1       | 2/2008           | Edwards et al.         | 2017/0233946 A1 | 8/2017    | Sealey et al.      |  |
| 2008/0076695 A1       | 3/2008           | Uitenbroek et al.      | 2017/0253422 A1 | 9/2017    | Anklam et al.      |  |
| 2008/0156450 A1       | 7/2008           | Klerelid et al.        |                 |           |                    |  |
| 2008/0199655 A1       | 8/2008           | Monnerie et al.        |                 |           |                    |  |
| 2008/0245498 A1       | 10/2008          | Ostendorf et al.       | CN              | 1138356 A | 12/1996            |  |
| 2008/0302493 A1       | 12/2008          | Boatman et al.         | CN              | 1207149 A | 2/1999             |  |
| 2008/0308247 A1       | 12/2008          | Ringer et al.          | CN              | 1244899 A | 2/2000             |  |

## FOREIGN PATENT DOCUMENTS

(56)

**References Cited**

## FOREIGN PATENT DOCUMENTS

|    |             |    |         |                                                                                                 |
|----|-------------|----|---------|-------------------------------------------------------------------------------------------------|
| CN | 1268559     | A  | 10/2000 | International Search Report for PCT/US15/64284 dated Feb. 11, 2016.                             |
| CN | 1377405     | A  | 10/2002 | Written Opinion of International Searching Authority for PCT/US15/64284 dated Feb. 11, 2016.    |
| CN | 2728254     | Y  | 9/2005  | International Search Report for PCT/US13/53593 dated Dec. 30, 2013.                             |
| DE | 4242539     | A1 | 8/1993  | Written Opinion of International Searching Authority for PCT/US13/53593 dated Dec. 30, 2013.    |
| EP | 0097036     | A2 | 12/1983 | International Search Report for PCT/US15/31411 dated Aug. 13, 2015.                             |
| EP | 0979895     | A1 | 2/2000  | Written Opinion of International Searching Authority for PCT/US15/31411 dated Aug. 13, 2015.    |
| EP | 1911574     | A1 | 1/2007  | International Search Report for PCT/US15/60398 dated Jan. 29, 2016.                             |
| EP | 1339915     | B1 | 7/2007  | Written Opinion of International Searching Authority for PCT/US15/60398 dated Jan. 29, 2016.    |
| EP | 2123826     | A2 | 5/2009  | International Search Report for PCT/US15/62483 dated May 6, 2016.                               |
| GB | 946093      | A  | 1/1964  | International Search Report for PCT/US16/56871 dated Jan. 12, 2017.                             |
| JP | 2013208298  | A  | 10/2013 | Written Opinion of International Searching Authority for PCT/US16/56871 dated Jan. 12, 2017.    |
| JP | 2014213138  | A  | 11/2014 | Written Opinion of International Searching Authority for PCT/US16/56871 dated Jan. 12, 2017.    |
| WO | 96/06223    | A1 | 2/1996  | International Search Report for PCT/US2016/057163 dated Dec. 23, 2016.                          |
| WO | 200382550   | A2 | 10/2003 | Written Opinion of International Searching Authority for PCT/US2016/057163 dated Dec. 23, 2016. |
| WO | 200445834   | A1 | 6/2004  | International Search Report for PCT/US2017/029890 dated Jul. 14, 2017.                          |
| WO | 2007070145  | A1 | 6/2007  | Written Opinion of International Searching Authority for PCT/US2017/029890 dated Jul. 14, 2017. |
| WO | 2008019702  | A1 | 2/2008  | International Search Report for PCT/US2017/032746 dated Aug. 7, 2017.                           |
| WO | 2009006709  | A1 | 1/2009  | Written Opinion of International Searching Authority for PCT/US2017/032746 dated Aug. 7, 2017.  |
| WO | 2009/061079 | A1 | 5/2009  | International Search Report for PCT/US17/17705 dated Jun. 9, 2017.                              |
| WO | 2009067079  | A1 | 5/2009  | Written Opinion of International Searching Authority for PCT/US17/17705 dated Jun. 9, 2017.     |
| WO | 2011028823  | A1 | 3/2011  | International Preliminary Report on Patentability of PCT/US2013/053593 dated Feb. 3, 2015.      |
| WO | 2012003360  | A2 | 1/2012  | Supplementary European Search Report of EP 13 82 6461 dated Apr. 1, 2016.                       |
| WO | 2013024297  | A1 | 2/2013  | * cited by examiner                                                                             |
| WO | 2013136471  | A1 | 9/2013  |                                                                                                 |
| WO | 2014/022848 | A1 | 2/2014  |                                                                                                 |
| WO | 201500755   | A1 | 1/2015  |                                                                                                 |
| WO | 2015/176063 | A1 | 11/2015 |                                                                                                 |
| WO | 2016/077594 | A1 | 5/2016  |                                                                                                 |
| WO | 2016/086019 | A1 | 6/2016  |                                                                                                 |
| WO | 2016/090242 | A1 | 6/2016  |                                                                                                 |
| WO | 2016/090364 | A1 | 6/2016  |                                                                                                 |
| WO | 2016085704  | A1 | 6/2016  |                                                                                                 |
| WO | 2017066465  | A1 | 4/2017  |                                                                                                 |
| WO | 2017066656  | A1 | 4/2017  |                                                                                                 |
| WO | 2017139786  | A1 | 8/2017  |                                                                                                 |

## OTHER PUBLICATIONS

International Search Report for PCT/US15/63986 dated Mar. 29, 2016.

Written Opinion of International Searching Authority for PCT/US15/63986 dated Mar. 29, 2016.



FIG. 1



FIG. 2



FIG. 3



FIG. 4

## SOFT THROUGH AIR DRIED TISSUE

## RELATED APPLICATION

This application is a divisional of U.S. patent application Ser. No. 15/182,391, filed Jun. 14, 2016 and entitled Soft Through Air Dried Tissue, which in turn is a continuation of U.S. patent application Ser. No. 14/534,631, filed Nov. 6, 2014 and entitled Soft Through Air Dried Tissue, issued as U.S. Pat. No. 9,382,666, which in turn is a divisional of U.S. patent application Ser. No. 13/837,685, filed Mar. 15, 2013 and entitled Soft Through Air Dried Tissue, issued as U.S. Pat. No. 8,968,517, which in turn claims priority to U.S. Provisional Application Ser. No. 61/679,337, filed Aug. 3, 2012 and entitled Soft Through Air Dried Tissue, the contents of these applications being incorporated herein by reference in their entirety.

## FIELD OF THE INVENTION

The present invention is directed to tissue, and in particular to a multilayer tissue including wet end additives.

## BACKGROUND

According to conventional tissue-making processes, a slurry of pulp mixture is fed to a headbox, where the mixture is laid onto a forming surface so as to form a web. The web is then dried using pressure and/or heat to form the finished tissue. Prior to drying, the pulp mixture is considered to be in the "wet end" of the tissue making process. Additives may be used in the wet end to impart a particular attribute or chemical state to the tissue. However, using additives in the wet end has some disadvantages. For example, a large amount of additive may be required in the pulp mixture to achieve the desired effect on the finished tissue, which in turn leads to increased cost and, in the case of wet end additive debonder, may actually reduce the tissue strength. In order to avoid drawbacks associated with wet end additives, agents, such as softeners, have been added topically after web formation.

The tissue web may be dried by transferring the web to a forming surface and then directing a flow of heated air onto the web. This process is known as through air drying (TAD). While topical softeners have been used in combination with through air dried tissue, the resulting products have had a tamped down or flattened surface profile. The flattened surface profile in turn hinders the cleaning ability of the tissue and limits the overall effectiveness of the softener.

## SUMMARY OF THE INVENTION

An object of the present invention is to provide a tissue manufacturing method that uses through air drying without compromising softness and cleaning ability of the resulting tissue.

Another object of the present invention is to provide a tissue manufacturing method that avoids the disadvantages associated with wet end additives, and in particular avoids the use of a large amount of additive to achieve the desired effect on the resulting tissue.

A multi-layer through air dried tissue according to an exemplary embodiment of the present invention comprises a first exterior layer, an interior layer and a second exterior layer. The interior layer includes a first wet end additive comprising an ionic surfactant and a second wet end additive comprising a non-ionic surfactant.

A multi-layer through air dried tissue according to another exemplary embodiment of the present invention comprises a first exterior layer comprised substantially of hardwood fibers, an interior layer comprised substantially of softwood fibers, and a second exterior layer comprised substantially of hardwood fibers. The interior layer includes a first wet end additive comprising an ionic surfactant and a second wet end additive comprising a non-ionic surfactant.

In at least one exemplary embodiment, the first exterior layer further comprises a wet end temporary wet strength additive.

In at least one exemplary embodiment, the first exterior layer further comprises a wet end dry strength additive.

In at least one exemplary embodiment, the second exterior layer further comprises a wet end dry strength additive.

In at least one exemplary embodiment, the second wet end additive comprises an ethoxylated vegetable oil.

In at least one exemplary embodiment, the second wet end additive comprises a combination of ethoxylated vegetable oils.

In at least one exemplary embodiment, the ratio by weight of the second wet end additive to the first wet end additive in the tissue is at least eight to one.

In at least one exemplary embodiment, the ratio by weight of the second wet end additive to the first wet end additive in the first interior layer is at most ninety to one.

In at least one exemplary embodiment, the tissue has a softness (hand feel) of at least 90.

In at least one exemplary embodiment, the tissue has a bulk softness of less than 10 TS7.

In at least one exemplary embodiment, the ionic surfactant comprises a debonder.

In at least one exemplary embodiment, the tissue has a tensile strength of at least 35 N/m, a softness of at least 90 and a basis weight of less than 25 gsm.

In at least one exemplary embodiment, the tissue has a tensile strength of at least 35 N/m, a softness of at least 90 and a caliper of less than 650 microns.

In at least one exemplary embodiment, the wet end temporary wet strength additive comprises glyoxalated polyacrylamide.

In at least one exemplary embodiment, the wet end dry strength additive comprises amphoteric starch.

In at least one exemplary embodiment, the first exterior layer further comprises a dry strength additive.

In at least one exemplary embodiment, the first and second exterior layers are substantially free of any surface deposited softener agents or lotions.

In at least one exemplary embodiment, at least one of the first or second exterior layers comprises a surface deposited softener agent or lotion.

In at least one exemplary embodiment, the tissue has a softness of at least 95.

In at least one exemplary embodiment, the non-ionic surfactant has a hydrophilic-lipophilic balance of less than 10, and preferably less than 8.5.

In at least one exemplary embodiment, the tissue may have a softness of at least 95.

In at least one exemplary embodiment, the first exterior layer is comprised of at least 75% by weight of hardwood fibers.

In at least one exemplary embodiment, the interior layer is comprised of at least 75% by weight of softwood fibers.

Other features and advantages of embodiments of the invention will become readily apparent from the following detailed description, the accompanying drawings and the appended claims.

## BRIEF DESCRIPTION OF THE DRAWINGS

Exemplary embodiments of the present invention will be described with references to the accompanying figures, wherein:

FIG. 1 is a schematic diagram of a three layer tissue in accordance with an exemplary embodiment of the present invention;

FIG. 2 shows a micrograph of the surface of a tissue according to an exemplary embodiment of the invention without a topical additive;

FIG. 3 shows a micrograph of the surface of a conventional through air dried tissue with a flattened surface texture; and

FIG. 4 is a block diagram of a system for manufacturing tissue according to an exemplary embodiment of the present invention.

## DETAILED DESCRIPTION

The present invention is directed to a soft tissue made with a combination of a wet end added ionic surfactant and a wet end added nonionic surfactant. The tissue may be made up of a number of layers, including exterior layers and an interior layer. In at least one exemplary embodiment, pulp mixes for each tissue layer are prepared individually.

FIG. 1 shows a three layer tissue, generally designated by reference number 1, according to an exemplary embodiment of the present invention. The tissue 1 has external layers 2 and 4 as well as an internal, core layer 3. External layer 2 is composed primarily of hardwood fibers 20 whereas external layer 4 and core layer 3 are composed of a combination of hardwood fibers 20 and softwood fibers 21. The internal core layer 3 includes an ionic surfactant functioning as a debonder 5 and a non-ionic surfactant functioning as a softener 6. As explained in further detail below, external layers 2 and 4 also include non-ionic surfactant that migrated from the internal core layer 3 during formation of the tissue 1. External layer 2 further includes a dry strength additive 7. External layer 4 further includes both a dry strength additive 7 and a temporary wet strength additive 8.

Pulp mixes for exterior layers of the tissue are prepared with a blend of primarily hardwood fibers. For example, the pulp mix for at least one exterior layer is a blend containing about 70 percent or greater hardwood fibers relative to the total percentage of fibers that make up the blend. As a further example, the pulp mix for at least one exterior layer is a blend containing about 90-100 percent hardwood fibers relative to the total percentage of fibers that make up the blend.

Pulp mixes for the interior layer of the tissue are prepared with a blend of primarily softwood fibers. For example, the pulp mix for the interior layer is a blend containing about 70 percent or greater softwood fibers relative to the total percentage of fibers that make up the blend. As a further example, the pulp mix for the interior layer is a blend containing about 90-100 percent softwood fibers relative to the total percentage of fibers that make up the blend.

As known in the art, pulp mixes are subjected to a dilution stage in which water is added to the mixes so as to form a slurry. After the dilution stage but prior to reaching the headbox, each of the pulp mixes are dewatered to obtain a thick stock of about 95% water. In an exemplary embodiment of the invention, wet end additives are introduced into the thick stock pulp mixes of at least the interior layer. In an exemplary embodiment, a non-ionic surfactant and an ionic surfactant are added to the pulp mix for the interior layer.

Suitable non-ionic surfactants have a hydrophilic-lipophilic balance of less than 10, and preferably less than or equal to 8.5. An exemplary non-ionic surfactant is an ethoxylated vegetable oil or a combination of two or more ethoxylated vegetable oils. Other exemplary non-ionic surfactants include ethylene oxide, propylene oxide adducts of fatty alcohols, alkylglycoside esters, and alkylethoxylated esters.

Suitable ionic surfactants include but are not limited to quaternary amines and cationic phospholipids. An exemplary ionic surfactant is 1,2-di(heptadecyl)-3-methyl-4,5-dihydroimidazol-3-ium methyl sulfate. Other exemplary ionic surfactants include (2-hydroxyethyl)methylbis[2-[(1-oxooctadecyl)oxy]ethyl]ammonium methyl sulfate, fatty dialkyl amine quaternary salts, mono fatty alkyl tertiary 15 amine salts, unsaturated fatty alkyl amine salts, linear alkyl sulfonates, alkyl-benzene sulfonates and trimethyl-3-[(1-oxooctadecyl)amino]propylammonium methyl sulfate.

In an exemplary embodiment, the ionic surfactant may function as a debonder while the non-ionic surfactant functions as a softener. Typically, the debonder operates by breaking bonds between fibers to provide flexibility, however an unwanted side effect is that the overall strength of the tissue can be reduced by excessive exposure to debonder. Typical debonders are quaternary amine compounds such as 25 trimethyl cocoammonium chloride, trymethyloleylammonium chloride, dimethyldi(hydrogenated-tallow)ammonium chloride and trimethylstearyl ammonium chloride.

After being added to the interior layer, the non-ionic surfactant (functioning as a softener) migrates through the 30 other layers of the tissue while the ionic surfactant (functioning as a debonder) stays relatively fixed within the interior layer. Since the debonder remains substantially within the interior layer of the tissue, softer hardwood fibers (that may have lacked sufficient tensile strength if treated 35 with a debonder) can be used for the exterior layers. Further, because only the interior of the tissue is treated, less debonder is required as compared to when the whole tissue is treated with debonder.

In an exemplary embodiment, the ratio of ionic surfactant 40 to non-ionic surfactant added to the pulp mix for the interior layer of the tissue is between 1:4 and 1:90 parts by weight and preferably about 1:8 parts by weight. In particular, when the ionic surfactant is a quaternary amine debonder, reducing the concentration relative to the amount of non-ionic 45 surfactant can lead to an improved tissue. Excess debonder, particularly when introduced as a wet end additive, can weaken the tissue, while an insufficient amount of debonder may not provide the tissue with sufficient flexibility. Because of the migration of the non-ionic surfactant to the exterior 50 layers of the tissue, the ratio of ionic surfactant to non-ionic surfactant in the core layer may be significantly lower in the actual tissue compared to the pulp mix.

In an exemplary embodiment, a dry strength additive is 55 added to the thick stock mix for at least one of the exterior layers. The dry strength additive may be, for example, amphoteric starch, added in a range of about 1 to 40 kg/ton. In another exemplary embodiment, a wet strength additive is added to the thick stock mix for at least one of the exterior 60 layers. The wet strength additive may be, for example, glyoxalated polyacrylamide, commonly known as GPAM, added in a range of about 0.25 to 5 kg/ton. In a further exemplary embodiment, both a dry strength additive, preferably amphoteric starch and a wet strength additive, preferably GPAM are added to one of the exterior layers. 65 Without being bound by theory, it is believed that the combination of both amphoteric starch and GPAM in a single layer when added as wet end additives provides a

synergistic effect with regard to strength of the finished tissue. Other exemplary temporary wet-strength agents include aldehyde functionalized cationic starch, aldehyde functionalized polyacrylamides, acrolein co-polymers and cis-hydroxyl polysaccharide (guar gum and locust bean gum) used in combination with any of the above mentioned compounds.

In addition to amphoteric starch, suitable dry strength additives may include but are not limited to glyoxalated polyacrylamide, cationic starch, carboxy methyl cellulose, guar gum, locust bean gum, cationic polyacrylamide, polyvinyl alcohol, anionic polyacrylamide or a combination thereof.

FIG. 4 is a block diagram of a system for manufacturing tissue, generally designated by reference number 100, according to an exemplary embodiment of the present invention. The system 100 includes an first exterior layer fan pump 102, a core layer fan pump 104, a second exterior layer fan pump 106, a headbox 108, a forming section 110, a drying section 112 and a calendar section 114. The first and second exterior layer fan pumps 102, 106 deliver the pulp mixes of the first and second external layers 2, 4 to the headbox 108, and the core layer fan pump 104 delivers the pulp mix of the core layer 3 to the headbox 108. As is known in the art, the headbox delivers a wet web of pulp onto a forming wire within the forming section 110. The wet web is laid on the forming wire with the core layer 3 disposed between the first and second external layers 2, 4.

After formation in the forming section 110, the partially dewatered web is transferred to the drying section 112. Within the drying section 112, the tissue of the present invention may be dried using conventional through air drying processes. In an exemplary embodiment, the tissue of the present invention is dried to a humidity of about 7 to 20% using a through air drier manufactured by Metso Corporation, of Helsinki, Finland. In another exemplary embodiment of the invention, two or more through air drying stages are used in series. Without being bound by theory, it is believed that the use of multiple drying stages improves uniformity in the tissue, thus reducing tears.

In an exemplary embodiment, the tissue of the present invention is patterned during the through air drying process. Such patterning can be achieved through the use of a TAD fabric, such as a G-weave (Prolux 003) or M-weave (Prolux 005) TAD fabric.

After the through air drying stage, the tissue of the present invention may be further dried in a second phase using a Yankee drying drum. In an exemplary embodiment, a creping adhesive is applied to the drum prior to the tissue contacting the drum. A creping blade is then used to remove the tissue from the Yankee drying drum. The tissue may then be calendered in a subsequent stage within the calendar section 114. According to an exemplary embodiment, calendering may be accomplished using a number of calendar rolls (not shown) that deliver a calendering pressure in the range of 0-100 pounds per linear inch (PLI). In general, increased calendering pressure is associated with reduced caliper and a smoother tissue surface.

According to an exemplary embodiment of the invention, a ceramic coated creping blade is used to remove the tissue from the Yankee drying drum. Ceramic coated creping blades result in reduced adhesive build up and aid in achieving higher run speeds. Without being bound by theory, it is believed that the ceramic coating of the creping blades provides a less adhesive surface than metal creping blades and is more resistant to edge wear that can lead to localized spots of adhesive accumulation. The ceramic creping blades

allow for a greater amount of creping adhesive to be used which in turn provides improved sheet integrity and faster run speeds.

In addition to the use of wet end additives, the tissue of the present invention may also be treated with topical or surface deposited additives. Examples of surface deposited additives include softeners for increasing fiber softness and skin lotions. Examples of topical softeners include but are not limited to quaternary ammonium compounds, including, but not limited to, the dialkyldimethylammonium salts (e.g. ditallowdimethylammonium chloride, ditallowdimethylammonium methyl sulfate, di(hydrogenated tallow)dimethyl ammonium chloride, etc.). Another class of chemical softening agents include the well-known organo-reactive polydimethyl siloxane ingredients, including amino functional polydimethyl siloxane, zinc stearate, aluminum stearate, sodium stearate, calcium stearate, magnesium stearate, spermaceti, and steryl oil.

The below discussed values for softness (i.e., hand feel (HF)), caliper and tensile strength of the inventive tissue were determined using the following test procedures:

#### Softness Testing

Softness of a tissue sheet was determined using a Tissue Softness Analyzer (TSA), available from emtec Electronic GmbH of Leipzig, Germany. A punch was used to cut out three 100 cm<sup>2</sup> round samples from the sheet. One of the samples was loaded into the TSA with the yankee side facing up. The sample was clamped in place and the TPII algorithm was selected from the list of available softness testing algorithms displayed by the TSA. After inputting parameters for the sample, the TSA measurement program was run. The test process was repeated for the remaining samples and the results for all the samples were averaged.

#### Caliper Testing

A Thwing-Albert ProGage 100 Thickness Tester, manufactured by Thwing Albert of West Berlin, N.J. was used for the caliper test. Eight 100 mm x 100 mm square samples were cut from a base sheet. Each sample was folded over on itself, with the rougher layer, typically corresponding air layer facing itself. The samples were then tested individually and the results were averaged to obtain a caliper result for the base sheet.

#### Tensile Strength Testing

An Instron 3343 tensile tester, manufactured by Instron of Norwood, Mass., with a 100N load cell and 25.4 mm rubber coated jaw faces was used for tensile strength measurement. Prior to measurement, the Instron 3343 tensile tester was calibrated. After calibration, 8 strips, each one inch by eight inches, were provided as samples for testing. One of the sample strips was placed in between the upper jaw faces and clamp, and then between the lower jaw faces and clamp. A tensile test was run on the sample strip. The test procedure was repeated until all the samples were tested. The values obtained for the eight sample strips were averaged to determine the tensile strength of the tissue.

Tissue according to exemplary embodiments of the present invention has an improved softness as compared to conventional tissue. Specifically, the tissue of the present invention may have a softness or hand feel (HF) of at least 90. In another exemplary embodiment, the tissue of the present invention may have a softness of at least 95.

In another exemplary embodiment, the tissue has a bulk softness of less than 10 TS7 (as tested by a TSA). In an exemplary embodiment, the tissue of the present invention also has a basis weight for each ply of less than 22 grams per

square meter. For such a soft, thin tissue the initial processing conditions may be defined so as to have a moisture content between 1.5 to 5%.

In another exemplary embodiment, the tissue of the present invention has a basis weight for each ply of at least 17 grams per square meter, more preferably at least 20 grams per square meter and most preferably at least 22 grams per square meter.

Tissue according to exemplary embodiments of the present invention has a good tensile strength in combination with improved softness and/or a lower basis weight or caliper as compared to conventional tissue. Without being bound by theory, it is believed that the process of the present invention allows the tissue to retain more strength, while still having superior softness without the need to increase the thickness or weight of the tissue. Specifically, the tissue of the present invention may have improved softness and/or strength while having a caliper of less than 650 microns.

Tissue according to exemplary embodiments of the present invention has a combination of improved softness with a high degree of uniformity of surface features. FIG. 2 shows a micrograph of the surface of a tissue according to an exemplary embodiment of the invention without a topical additive and FIG. 3 shows a micrograph of the surface of a conventional through air dried tissue with a flattened surface texture. The tissue of FIG. 2 has a high degree of uniformity in its surface profile, with regularly spaced features, whereas the tissue of FIG. 3 has flattened regions and a nonuniform profile.

The tissue of the present invention may also be calendered or treated with a topical softening agent to alter the surface profile. In exemplary embodiments, the surface profile can be made smoother by calendering or through the use of a topical softening agent. The surface profile may also be made rougher via microtexturing.

The following examples are provided to further illustrate the invention.

#### EXAMPLE 1

Through air dried tissue was produced with a three layer headbox and a 005 Albany TAD fabric. The flow to each layer of the headbox was about 33% of the total sheet. The three layers of the finished tissue from top to bottom were labeled as air, core and dry. The air layer is the outer layer that is placed on the TAD fabric, the dry layer is the outer layer that is closest to the surface of the Yankee dryer and the core is the center section of the tissue. The tissue was produced with 45% eucalyptus fiber in the air layer, 50% eucalyptus fiber in the core layer and 100% eucalyptus fiber in the dry layer. Headbox pH was controlled to 7.0 by addition of a caustic to the thick stock before the fan pumps for all samples.

Roll size was about 10,000 meters long. The number of sheet-breaks per roll was determined by detecting the number of breaks in the sheet per every 10,000 meters of linear (MD-machine direction) sheet run.

The tissue according to Example 1 was produced with addition of a temporary wet strength additive, Hercobond 1194 (Ashland, 500 Hercules Road, Wilmington Del., 19808) to the air layer, a dry strength additive, Redibond 2038 (Corn Products, 10 Finderne Avenue, Bridgewater, N.J. 08807) split 75% to the air layer, 25% to the dry layer, and a softener/debonder, T526 (EKA Chemicals Inc., 1775 West Oak Commons Court, Marietta, Ga., 30062) added in combination to the core layer. The T526 is a softener/debonder combination with a quaternary amine concentration below 20%.

#### EXAMPLE 2

Example 2 was produced with the same conditions as Example 1, but chemical addition rates were changed. Specifically, the amount of dry strength additive (Redibond 2038) was increased from 5.0 kg/ton to 10.0 kg/ton and the amount of softener/debonder (T526) was increased from 2.0 kg/ton to 3.6 kg/ton.

#### EXAMPLE 3

Example 3 was produced with the same conditions as Example 1 except with T526 added to the dry layer.

#### EXAMPLE 4

Example 4 was produced with the same conditions as Example 1 except for the addition of a debonder having a high quaternary amine concentration (>20%) to the core layer. The debonder was F509HA (manufactured by EKA Chemicals Inc., 1775 West Oak Commons Court, Marietta, Ga., 30062).

#### COMPARATIVE EXAMPLE 1

Comparative Example 1 was produced with the same conditions as Example 1 except that wet end additives were not used

Table 1 shows performance data and chemical dose information for the TAD basesheet of Examples 1-4 and Comparative Example 1. The basis weight (BW) of each Example was about 20.7 GSM.

TABLE 1

| Sample                   | HF <sup>1</sup> | MD/CD<br>Tensile<br>n/m <sup>2</sup> | Lint<br>Value <sup>3</sup> | Hercobond<br>D1194<br>kg/ton | Redibond<br>2038<br>kg/ton | (temporary<br>wet<br>strength<br>additive) | (temporary<br>dry<br>strength<br>additive) | EKA T526<br>(Softener/debonder)<br>kg/ton | Sheet-<br>breaks<br>per<br>roll |
|--------------------------|-----------------|--------------------------------------|----------------------------|------------------------------|----------------------------|--------------------------------------------|--------------------------------------------|-------------------------------------------|---------------------------------|
| Comparative<br>Example 1 | 93.8            | 55/27                                | 11.5                       | 0                            | 0                          |                                            |                                            | 0                                         | 3                               |
| Example 1                | 98.2            | 54/34                                | 9.0                        | 1.25                         | 5.0                        |                                            |                                            | 2.0                                       | 0                               |
| Example 2                | 95.1            | 56/38                                | 7.5                        | 1.25                         | 10                         |                                            |                                            | 3.6                                       | 0                               |

TABLE 1-continued

| Sample    | HF <sup>1</sup> | MD/CD Tensile n/m <sup>2</sup> | Lint Value <sup>3</sup> | Hercobond D1194 kg/ton (temporary wet strength additive) | Redibond 2038 kg/ton (temporary dry strength additive) | EKA T526 kg/ton (Softener/debonder) | Sheet-breaks per roll |
|-----------|-----------------|--------------------------------|-------------------------|----------------------------------------------------------|--------------------------------------------------------|-------------------------------------|-----------------------|
| Example 3 | 91.5            | 57/39                          | 12.0                    | 1.25                                                     | 5.0                                                    | 2.0                                 | 1                     |
| Example 4 | 90.5            | 55/35                          | 9.8                     | 1.25                                                     | 10                                                     | 0.81 (F509HA)                       | 0                     |

<sup>1</sup>All HF values are from single ply basesheet samples with dry side surface up.

<sup>2</sup>Basesheet single ply data.

<sup>3</sup>Post converted two ply product tested.

Examples 1 and 2 had a much higher hand-feel (HF) with lower lint value and improved machine efficiency compared to Comparative Example 1. Of note, these improved parameters were achieved while maintaining the same sheet MD/CD tensile range for both Examples 1 and 2 as in Comparative Example 1. The wet end chemical additives of Example 1 significantly improved product softness. Example 2 is a further improvement over Example 1 with a reduced lint value. This improvement in Example 2 was achieved by increasing the Redibond 2038 and T526 dose.

Softness as determined by the TSA was significantly reduced when softener/debonder was added to the dry layer (Example 3) and when a tissue debonder having a higher quaternary amine concentration was added to the core layer (Example 4). The preferred option is to add a combination of softener/debonder to core layer which allows the softener to migrate to surface layers and adjust chemical bonding in the dry layer to control product lint level (Example 1).

The tissue of the present invention also exhibits an improved surface profile that provides for improved product consistency and fewer defects that may otherwise cause sheet breaks. Specifically, the roughness of tissue can be characterized using two values, Pa (Average Primary Amplitude) and Wc (Average Peak to Valley Waviness). Pa is a commonly used roughness parameter and is computed as the average distance between each roughness profile point and the meanline. Wc is computed as the average peak height plus the average valley depth (both taken as positive values) relative to the meanline. As described in more detail below, the tissue of the present invention is measured to have Pa and Wc values that are both low and relatively uniform compared to conventional TAD tissue products.

The below discussed values for Pa and Wc of the inventive tissue were determined using the following test procedures:

#### Pa and Wc Testing

Ten samples of each tissue to be tested were prepared, with each sample being a 10 cm by 10 cm strip. Each sample was mounted and held in place with weights. Each sample was placed into a Marsurf GD 120 profilometer, available from Mahr Federal Instruments of Gottingen, Germany, and oriented in the CD direction. A 5  $\mu$ m tip was used for the profilometer. Twenty scans were run on the profilometer per sample (ten in the forwards direction and ten in the backwards direction). The reverse scans were performed by turning the sample 180 degrees prior to scanning. Each scan covered a 30 mm length. The collected surface profile data was then transferred to a computer running OmniSurf analysis software, available from Digital Metrology Solutions, Inc. of Columbus, Ind., USA. The roughness profile setting for the OmniSurf software was set with a short filter low range of 25 microns and a short filter high range of 0.8 mm.

The waviness profile setting of the OmniSurf software was set to a low range of 0.8 mm. For each sample, values for Pa (Average Primary Amplitude) and Wc (Average Peak to Valley Waviness) were calculated by the Omni Surf software. The calculated values of Pa and Wc for all twenty scans were averaged to obtain Pa and Wc values for each tissue sample. The standard deviation of the individual sample Pa and Wc values were also calculated.

The following examples are provided to further illustrate the invention.

#### EXAMPLE 5

Two plies were produced, with each ply being equivalent to the three-layer structure formed in Example 1. The two plies were then embossed together to form a finished tissue product.

#### COMPARATIVE EXAMPLE 2

Two plies were produced and embossed together as in Example 5, except that wet end additives were not used.

Table 2 shows the Pa and Pa standard deviation of several commercial products, Example 5, and Comparative Example 2 and 3.

TABLE 2

| 45                             | SAMPLE   | Pa       | S.D                  | LOCATION PURCHASED | DATE PURCHASED |
|--------------------------------|----------|----------|----------------------|--------------------|----------------|
| Charmin Basic                  | 82.58245 | 9.038986 | Wal-Mart - Anderson  | Jul-12             |                |
| Charmin Strong                 | 57.03765 | 8.130364 | Target - Anderson SC | Jul-12             |                |
| Charmin Soft                   | 47.3826  | 9.72459  | Wal-Mart - Anderson  | Jun-12             |                |
| Charmin Soft                   | 79.33375 | 9.620164 | Wal-Mart - Anderson  | Jan-12             |                |
| Charmin Strong                 | 70.6232  | 11.32204 | Wal-Mart - Anderson  | Jan-12             |                |
| 55 Cottonelle Clean Care       | 100.9827 | 11.21668 | Wal-Mart - Anderson  | Jan-12             |                |
| Cottonelle Ultra               | 90.5762  | 13.82119 | Wal-Mart -           | Jan-12             |                |
| Comfort Care                   |          |          | Anderson             |                    |                |
| Target UP & UP Soft and Strong | 65.9598  | 12.45098 | Target - Anderson SC | Sep-12             |                |
| Comparative Example 2          | 86.2806  | 9.46203  |                      |                    |                |
| Example 5                      | 41.66115 | 2.19889  |                      |                    |                |

Table 3 shows the Wc and Wc standard deviation of several commercial products, Example 5, and Comparative Example 2.

## 11

TABLE 3

| SAMPLE                                                            | Wc        | S.D      | LOCATION PURCHASED   | DATE PURCHASED |
|-------------------------------------------------------------------|-----------|----------|----------------------|----------------|
| Charmin Basic                                                     | 181.2485  | 31.50583 | Wal-Mart - Anderson  | Jul-12         |
| Charmin Strong                                                    | 163.4448  | 37.6021  | Target - Anderson SC | Jul-12         |
| Charmin Soft                                                      | 147.54785 | 38.41011 | Wal-Mart - Anderson  | Jun-12         |
| Charmin Soft                                                      | 185.51195 | 30.68851 | Wal-Mart - Anderson  | Jan-12         |
| Charmin Strong                                                    | 216.1236  | 49.08633 | Wal-Mart - Anderson  | Jan-12         |
| Cottonelle                                                        | 307.39355 | 34.06675 | Wal-Mart - Anderson  | Jan-12         |
| Clean Care Cottonelle Ultra                                       | 286.33735 | 51.90506 | Wal-Mart - Anderson  | Jan-12         |
| Comfort Care Target UP & UP Soft and Strong Comparative Example 2 | 228.9568  | 59.57366 | Target - Anderson SC | Sep-12         |
| Example 5                                                         | 239.8652  | 54.96261 |                      |                |
|                                                                   | 123.41615 | 14.97908 |                      |                |

Tables 1 and 2 show the improved surface roughness characteristics of the inventive tissue as compared to commercially available products as well as similar tissue products that were not produced with wet end additives. Specifically, the tissue according to various exemplary embodiments of the present invention has an average Wc value of 140 or less, and more preferably 135 or less, with a Wc standard deviation (i.e., Waviness Uniformity) of 27 or less. Further, the tissue according to various exemplary embodiments of the present invention has an average Pa value of 50 or less, with a Wc standard deviation (i.e., Amplitude Uniformity) of 8 or less.

As known in the art, the tissue web is subjected to a converting process at or near the end of the web forming line to improve the characteristics of the web and/or to convert the web into finished products. On the converting line, the tissue web may be unwound, printed, embossed and rewound. According to an exemplary embodiment of the invention, the paper web on the converting lines may be treated with corona discharge before the embossing section. This treatment may be applied to the top ply and/or bottom ply. Nano cellulose fibers (NCF), nano crystalline cellulose (NCC), micro-fibrillated cellulose (MCF) and other shaped natural and synthetic fibers may be blown on to the paper web using a blower system immediately after corona treatment. This enables the nano-fibers to adsorb on to the paper web through electro-static interactions.

As discussed, according to an exemplary embodiment of the invention, a debonder is added to at least the interior layer as a wet end additive. The debonder provides flexibility to the finished tissue product. However, the debonder also reduces the strength of the tissue web, which at times may result in sheet breaks during the manufacturing process. The relative softness of the tissue web results in inefficiencies in the rewind process that must be performed in order to correct a sheet break. Accordingly, as shown in FIG. 4, in an exemplary embodiment of the present invention, a switching valve 120 is used to control delivery of the debonder as a wet-end additive to the interior layer. In particular, when a sheet break is detected using, for example,

## 12

conventional sheet break detection sensors, the switching valve 120 may be controlled to prevent further delivery of the debonder. This results in less flexibility and increased strength at the portion of the tissue web to be rewound, thereby allowing for a more efficient rewind process. Once the rewind process is completed, the switching valve may be opened to continue delivery of the debonder.

In addition to the use of a sheet break detection sensor, the switching valve 120 may also be controlled during turn up, the process whereby the tissue web is one transferred from on roll to another. The turn up process can result in higher stresses on the tissue web than normal operation, thus increasing the chance of sheet breaks. The switching valve 120 is turned off prior to turn up, thus increasing the strength of the tissue web. After the tissue web has begun winding on a new roll, the switching valve 120 is turned on again. The resulting roll of basesheet material thus has a section of higher strength tissue web at the center of the roll and may have a section of higher strength tissue on the outside of the roll. During finishing, the exterior section of higher strength tissue is removed and recycled. The interior section of higher strength tissue is not used to make a finished tissue. Thus, only the portion of the roll of basesheet tissue containing debonder is used to make finished tissue.

Now that embodiments of the present invention have been shown and described in detail, various modifications and improvements thereon will become readily apparent to those skilled in the art. Accordingly, the spirit and scope of the present invention is to be construed broadly and not limited by the foregoing specification.

What is claimed is:

1. A system for making tissue, comprising:  
a mixing section that provides a pulp mix, the mixing section including a wet-end adding section that delivers a wet-end additive to the pulp mix at a first point in a process for manufacturing tissue;
2. The system of claim 1, wherein the wet-end adding section forms after the first point in the process a wet web from the pulp mix provided by the mixing section;
3. The system of claim 2, wherein the wet web is dried into a basesheet of tissue;
4. The system of claim 3, wherein the basesheet is wound onto a roll; and
5. The system of claim 4, wherein a sensor detects a break in the basesheet tissue; wherein operation of the wet-end adding section is controlled by the sensor so that delivery of the wet-end additive to the pulp mix is prevented at the first point in response to the sensor detecting a break in the basesheet tissue.

50 2. The system of claim 1, wherein the wet-end adding section comprises a switching valve that is coupled to the sensor and through which the wet-end additive is added to the pulp mix.

3. The system of claim 2, wherein the switching valve is responsive to the sensor.

4. The system of claim 3, wherein the switching valve is closed when the sensor detects a break in the tissue web.

5. The system of claim 1, wherein the wet-end additive comprises a debonder.

60 6. The system of claim 1, wherein the forming section comprises a three layer headbox and the pulp mix is formed into an interior layer of the wet web.

\* \* \* \* \*